

T. E. MURRAY.  
METHOD OF MAKING A MOLDED CONDUIT.  
APPLICATION FILED JAN. 6, 1921.

1,387,067.

Patented Aug. 9, 1921.

Fig:1.



Fig:2.



Inventor  
Thomas E. Murray  
By his Attorney  
Carl Benjamin

# UNITED STATES PATENT OFFICE.

THOMAS E. MURRAY, OF BROOKLYN, NEW YORK.

## METHOD OF MAKING A MOLDED CONDUIT.

1,387,067.

Specification of Letters Patent. Patented Aug. 9, 1921.

Application filed January 6, 1921. Serial No. 435,408.

*To all whom it may concern:*

Be it known that I, THOMAS E. MURRAY, a citizen of the United States, residing at Brooklyn, in the county of Kings and State 5 of New York, have invented a certain new and useful Improvement in Methods of Making a Molded Conduit, of which the following is a specification.

Conduits of cement or like plastic material have been molded upon a spiral core of wire or the like provided with a cover or wrapping of paper or similar flexible material. When the core is withdrawn after the cement has hardened, the paper is left in the 15 bore. Where the conduit is used to convey water or other liquid, the paper is softened and eventually detached, and thus becomes washed into elbows, valves or smaller branch pipes—in all cases more or less choking these 20 and so stopping or impairing the flow.

My present invention is a method of molding said conduits so that the paper cover becomes a lining permanently affixed to the surface of the bore and which cannot be 25 loosened or washed away, thus avoiding the above-described difficulty. My said method consists in the steps performed in the order stated more particularly in the claim.

In the accompanying drawing—

30 Figure 1 represents in longitudinal section a portion of the conduit and core therein. Fig. 2 is a similar view of said conduit after the removal of the core.

Similar numbers of reference indicate like 35 parts.

In performing my method, I first make a spiral core 1 of wire or strip metal. Upon said core I apply, preferably by wrapping,

a cover 2 of paper or similar flexible sheet material. To this cover I next apply a coating 3 of pitch or other viscid adhesive material which will harden. While the pitch coating is still viscid, I apply thereto plastic cement or concrete 4 to form the conduit body, and allow said plastic material to become hard. Finally, I withdraw the core 1. The cover 2 remains firmly held by the pitch coating and said coating in turn unites with the cement surrounding it, so that the cement, the cover and the pitch form a solid 50 hard mass, of which the cover forms a fixed lining having a smooth inner surface, and which is not washed away nor loosened by liquid flow in the conduit. The said mass, besides, is wholly of insulating material, 55 thus adapting the conduit to the conveyance of electrical conductors. Where the cement or concrete is at all porous, the pitch layer renders it impervious to both gases and liquids. 60

I claim:

The method of making a molded conduit, which consists in, first, producing a spiral metal core; second, covering said core with flexible material; third, applying to said 65 cover a coating of adhesive material; fourth, forming upon said coated core the conduit body of plastic material and allowing the same to harden, and fifth, withdrawing said spiral core. 70

In testimony whereof I have affixed my signature in presence of two witnesses.

THOMAS E. MURRAY.

Witnesses:

GERTRUDE T. PORTER,  
MAY T. McGARRY.